

## UNITED STATES PATENT OFFICE

2,179,371

## DYEING TEXTILE MATERIALS

Colver P. Dyer, Winchester, Mass., assignor, by  
mesne assignments, to Monsanto Chemical  
Company, a corporation of Delaware

No Drawing. Application May 29, 1936,  
Serial No. 82,523

7 Claims. (Cl. 8—54)

The present invention relates to the dyeing of fibrous materials and it has particular relation to the dyeing of such materials as wool or leather which are composed of proteinous fibers or filaments.

5 The main objects of the invention are to provide:

A material for obtaining so-called "level" or uniform impregnation of the fibers by the dye.

10 A material for producing uniformity of color in "union" and "speck" dyeing. These and other objects will be apparent from consideration of the following specifications and the appended claims.

15 In the dyeing of wools, leathers and similar materials containing proteinous substances as essential constituents of the fibers, difficulty is experienced by reason of the fact that some dyes do not uniformly penetrate into the fibers and as a result more or less mottled, streaky, uneven effects are obtained. Such dyes are termed "un-level". This is especially true in the case of certain cheap dyes, some of which are extremely resistant to fading and discoloration under the influence of washing, exposure to light, and perspiration, and which, if they were "level", would have gone onto much wider use than they have heretofore enjoyed. In consequence, dyers have been forced to resort to the use of much more expensive materials, some of which were also characterized by low resistance to fading and discoloration by the above indicated agencies. It has been proposed to overcome the "un-level" effects of the first mentioned class of dyes by 30 conducting dyeing operations in the presence of certain agents, notably Glauber's salt. While these agents produced some improvement, they were never entirely satisfactory.

35 Difficulty has also been experienced in the dyeing of mixed fabrics composed of threads or fibers of wool interspersed with threads or bits of cotton or the like cellulosic materials, because the wool tended to absorb dye more readily than the cellulosic fibers and as a result uniform color of the finished product could not be obtained.

40 The present invention is based upon the discovery that certain reaction products of formaldehyde and sulfonated aromatic compounds, such as naphthalene, when incorporated into dye 45 solutions have the property of producing highly uniform impregnation of proteinous fibers composing such materials as wool, leather or the like and excellent "level" effects are obtained even with dye compounds which have heretofore 50 been so "unlevel" in characteristics as practically

to inhibit their use at least in the finer grades of materials. Great uniformity of color is also produced upon textile materials consisting of wool or similar proteinous materials mixed with cotton or similar cellulosic materials. It thus becomes 5 possible to dye mixed fabrics to substantially uniform color by application of the foregoing reaction products.

Certain condensation products of naphthalene sulfonic acid and formaldehyde have heretofore 10 been suggested as synthetic tanning agents and are termed syntans. While the compounds preferred in the practice of the present invention are related to the syntans, they are characterized by higher molecular weight and a slower rate of 15 solution (in the undiluted state) in water than the ordinary synthetic tanning agents. They, also, have the power of reducing the rate of absorption of dyes from baths by certain materials, notably wool, to a much greater degree 20 than the ordinary synthetic tanning agents. These characteristics constitute convenient tests for distinguishing applicant's preferred material from the ordinary synthetic tanning agents.

The new dye retarding compounds are readily 25 obtained by condensing sulfonated aromatic compounds such as naphthalene with formaldehyde. Usually the degree of sulfonation should correspond at least to the mono-sulfonic acid derivative of the aromatic compound and preferably it should approach that theoretically required for di-sulfonation. Very satisfactory results are obtained when the sulfo group is combined in the ratio of approximately 1.6 or 1.7 30 mols per mol. of naphthalene. This may be obtained by heating two parts by weight of 100% 35 sulfuric acid with one part of naphthalene at a temperature of 140° C. for a period of three hours. The sulfonation of naphthalene and similar organic compounds by means of concentrated 40 sulfuric acid or chlor-sulfonic acid is well known to those skilled in the art and detailed discussion is not deemed to be necessary. The sulfonation of naphthalene when cool is admixed in a closed vessel with 12 liters of water per 22 kilos of 45 original naphthalene, and formaldehyde of 37% by weight concentration in a suitable ratio. Ratios of from .47 to about 1 part of formaldehyde to 1 part of original naphthalene and even 50 somewhat higher or lower may be used but the ratio of about 1 part of naphthalene to 0.7 part formaldehyde is deemed to be preferable. The addition of formaldehyde requires about four hours and the sulfonic acid solution is maintained during this period at a temperature of 55

about 80° C. After all of the formaldehyde has been added, the temperature is raised to and maintained at 100° C. for a period of two and one-half hours. A four kilo portion of water 5 is then added and reaction is continued as a final stage for six to twenty hours longer. Temperature differences greater than 2° C. in various parts of the bath are to be avoided during the reaction.

10 In the preparation of the product, the proportion of water incorporated, during the reaction may vary within wide limits. For example, amounts of 12 or more kilograms may be added preliminary to the final stage of reaction, if the 15 time and temperature of reaction are correspondingly adjusted. If the amount of water is materially reduced, it is desirable to reduce the reaction temperature in order to slow down the rate of reaction sufficiently to admit of proper 20 tests for determination of the degree of reaction. The following constitutes a suitable test for determination of the suitability of the material for use in dyeing operations:

25 Take a sample equivalent to .76 gram of the original naphthalene, which sample, if the material is prepared by the foregoing directions, should weigh about 3.5 grams. The sample should be added with agitation to 1500 cc. of water having a temperature of 90° C. The time 30 required for the material to pass into solution is found to vary with the degree of reaction of the product. For example, as the reaction progresses, it will be observed that the time required for the product to dissolve will increase along 35 a curve that reaches a peak of about twenty minutes. The solubility then gradually decreases to a minimum of six minutes. A product of optimum properties should pass into solution within a period of about four to seven minutes or slightly less, but products dissolving within about ten minutes are also satisfactory for many purposes.

40 At the end of the reaction, soda ash, dry or as a 20% solution, is added to the hot mixture 45 to neutralize it and the neutralized solution is diluted with water to 8.25 liters per kilo of naphthalene employed. A product of relatively high viscosity is obtained. This viscosity is to some extent an indicator of the degree of reaction obtained. For example, a material which 50 is satisfactory for use in dyeing processes generally should at normal room temperatures be at least about as thick and viscous as heavy and relatively cold machine oil and, preferably, it is 55 of almost jelly-like consistency almost capable of slicing and standing up as a tremulous mass roughly resembling ordinary edible gelatin when poured from a mold. It is found that where the reaction is discontinued before the oil-like 60 consistency is reached that the levelling action upon the absorption of dyes is relatively low. However, if the reaction between the aromatic sulfonic acid and the formaldehyde is continued over too long a period or at too high a temperature 65 the material enters into a relatively insoluble stage and is then impracticable for use in ordinary dyeing operation.

70 An additional test for determination of the suitability of the product for use in dye levelling operations, involves determination of its power to slow up the rate of dye absorption by woolen goods. This test may conveniently be conducted as follows: Prepare a test bath containing 3% by weight of Sulfone Acid, Blue R designated 75 in the Color Index of 1934, published by the

American Association of Textile Chemists as "208". The bath should also contain 5% of 28% acetic acid along with the dye levelling compound in appropriate amount (e. g. 20%) based upon the weight of the test wool to be dyed. This amount of material is equivalent to 1.5% of naphthalene upon a like basis.

5 The wool sample equals 2.2% by weight of the water in the bath. The temperature of the bath is initially about 50° C. It is then brought up to a temperature of 94° C. over a period of fifteen minutes. Finally, the dye bath is maintained at a boiling temperature for a period of 10 to 120 minutes and during this time samples of the bath are taken at ten minute intervals and titrated in accordance with standard 15 procedure with titanium trichloride solution. The degree of dye fixation was determined by the difference in titration between a given sample and a test run upon the solution prior to the 20 addition of the dye absorbing goods. The following table gives the results of a test of satisfactory material and, for purposes of comparison, the results of similar tests conducted with similar dye solutions but containing no leveller (blank). In the table, the results are expressed as time in minutes required for a given amount 25 of dye to be absorbed into the woolen test cloth.

| Percent dye absorbed from bath | Dye soln.<br>blank | Dye soln.+20%<br>new condensa-<br>tion product | 30 |
|--------------------------------|--------------------|------------------------------------------------|----|
| 10                             | 9                  | 10                                             |    |
| 20                             | 13                 | 23                                             | 10 |
| 30                             | 16                 | 33                                             | 15 |
| 40                             | 18                 | 41                                             | 20 |
| 50                             | 20                 | 48                                             | 25 |

It will be noted that with the highly condensed product constituting the subject matter of the present invention, the time required to obtain 40 40% absorption of the dye is more than twice as great as that required to obtain an equal degree of absorption in the blank.

45 In the dyeing of wool, the above described material may be employed with satisfactory results over a wide range of proportions. As little as 0.3 of 1% will in some cases produce notable levelling effects and as much as 30% or even more may in some cases be employed. Probably best results are obtained by employing from 10 50 to 20%. These values are based upon the weight of wool contained in the fabrics which are to be treated. The proportion of water employed to make up the dye solution, of course, may vary but good results are obtainable by using water 55 equal in weight to about 20 to 45 times the weight of the cloth. The proportion of dye, of course, will depend upon the intensity of the shade desired, the nature of the dye employed and various other factors as well understood by 60 those skilled in the art.

65 Application of the condensation products is not restricted to the particular dye mentioned above but may be made to numerous other dyes. The following constitutes a list of some of the 65 dyes to which application of the compounds has been made. The numbers given are those employed in the Color Index of 1934 published by the American Association of Textile Chemists and Colorists.

|      |      |     |    |
|------|------|-----|----|
| 252  | 79   | 304 | 70 |
| 179  | 1054 | 670 |    |
| 246  | 53   | 419 |    |
| 114  | 666  | 430 |    |
| 1078 | 833  | 138 | 75 |

5 Sulfonated benzene, toluene, xylene, diphenyl and propylated or butylated benzene, or naphthalene and phenol and alpha or beta naphthol may be substituted for sulfonated naphthalene and condensed with formaldehyde to provide materials which are also contemplated by the present invention. Sulfonation may follow condensation of the aromatic compound with formaldehyde. Other aldehydic agents than formaldehyde, e. g. hexamethylenetetramine acetaldehyde and furfural may be employed.

10 The levelling agent may be employed in re-dyeing operations such as "speck" dyeing in which a readily dyeable material such as wool, that contains some more difficultly dyeable fibers such as cellulose, is first subjected to the action of an ordinary dye with or without a leveller and is then re-dyed in an additional bath especially suitable for coloring the cellulosic fibers. If the latter 15 bath contains the levelling agent disclosed herein, the cellulose fibers will be dyed to approximately the same shade as the wool. If the leveller is omitted, the wool will be much more strongly colored than the cotton.

20 25 Although only the preferred forms of the invention have been shown and described, it will be apparent to those skilled in the art that the invention is not limited to these specific forms but numerous modifications may be made therein without departure from the spirit of the invention or the scope of the appended claims.

30 What I claim is:

35 1. A dye levelling compound for retarding the fixation of dyes to proteinous materials comprising a reaction product of formaldehyde and naphthalene sulfonic acid, an unneutralized 3.5 gram sample of which, when it is of such water content as to contain .76 gram of naphthalene, will dissolve in 1,500 cc. of water at 90° C. within a period 40 of approximately six to thirty minutes.

45 2. A method of promoting uniform dye impregnation of woolen textile material with acid dyes comprising incorporating into the bath employed in dyeing the material, a condensation product of naphthalene sulfonic acid and formaldehyde, said condensation product being semi-gelatinous when admixed with 8.4 parts of water per unit weight of naphthalene introduced into the reaction product, and further characterized by the ability to retard the 50 fixation of acid dyes to the textile material.

55 3. A method of promoting level dyeing of proteinous fibers with acid dyes which comprises introducing into the bath employed in the dyeing operation, a condensation product of naphthalene sulfonic acid and formaldehyde, said con-

densing product being characterized by the ability to reduce the rate of dye-absorption to approximately 85% or less of the normal rate when introduced into a bath of normally unlevel acid dyestuff and further characterized in that 5 said condensation product is semi-gelatinous when admixed with 8.4 parts of water per unit weight of naphthalene introduced into the reaction product.

10 4. A method of promoting uniform dye impregnation of woolen textile material with acid dyes, which comprises incorporating into the bath employed in dyeing the material, a condensation product of naphthalene sulfonic acid containing sulfo groups substantially in excess of mono 15 molar ratio with respect to the naphthalene and formaldehyde, the formaldehyde being in a ratio of from .5 to .7, with respect to the naphthalene, said product being semi-gelatinous when admixed with 8.4 parts of water per unit weight of naphthalene introduced into the reaction product, and further characterized by the ability to retard the 20 fixation of acid dyes to the textile material.

25 5. A method of promoting level dyeing of proteinous fibers with acid dyes which comprises introducing into the bath employed in the dyeing operation a reaction product of naphthalene sulfonic acid with from .7 to 1 part by weight of 37% formaldehyde, said product being substantially free of tanning properties, and further characterized by the ability to retard the fixation of 30 acid dyes to the fibers and by the fact that an unneutralized 3.5 gram sample thereof when it is of such water content as to contain .76 gram of 35 naphthalene will dissolve in 1500 cc. of water at 90° C. within a period of approximately 6 to 30 minutes.

40 6. A method of promoting level dyeing of union fabrics with acid dyes which comprises introducing into the bath employed in the dyeing operation a reaction product of formaldehyde and naphthalene sulfonic acid, an unneutralized 3.5 gram sample of which, when it is of such water content as to contain .76 gram of naphthalene, will dissolve in 1500 cc. of water at 90° C. within 45 a period of approximately six to thirty minutes.

45 7. A dye levelling compound comprising a reaction product of naphthalene sulfonic acid with formaldehyde, the formaldehyde being in a ratio of not less than .47 part of 37% concentration 50 with respect to the naphthalene, said condensation product being semi-gelatinous when admixed with 8.4 parts of water per unit weight of naphthalene introduced into the reaction product.

COLVER P. DYER. 55